

Nov. 22, 1960

J. S. KOUVEL ET AL

2,961,360

MAGNETS HAVING ONE EASY DIRECTION OF MAGNETIZATION

Filed Dec. 1, 1958

Fig. 1.



Fig. 2.



Fig. 3.



Inventors:  
James S. Kouvel;  
Charles D. Graham, Jr.

by *Charles J. Worth*  
Their Attorney.

## 1

2,961,360

MAGNETS HAVING ONE EASY DIRECTION  
OF MAGNETIZATION

James S. Kouvel, Albany, and Charles D. Graham, Jr., Schenectady, N.Y., assignors to General Electric Company, a corporation of New York

Filed Dec. 1, 1958, Ser. No. 777,324

3 Claims. (Cl. 148—103)

This invention relates to permanent magnets and more particularly to permanent magnets having one easy direction of magnetization and to a method for producing such magnets.

Previously known magnetic materials have been most readily magnetized along one particular axis and have been equally readily magnetizable in either direction along that axis. The magnetic properties of these materials have been measured and evaluated by several methods, perhaps the best known being the graphical representation of the hysteresis loop obtained when a magnetic field is applied to the magnetic material in such a manner as to cyclically reverse polarity. Since magnetic properties have been symmetrically reversible, both quantitatively and qualitatively with respect to the axis of magnetization, they also have at least two stable positions in a strong magnetic field.

While existing magnetic materials have generally proven acceptable for use in most situations, the increasing use of electronic and electrical apparatus under unusual environmental conditions has resulted in a need for components having particular properties when subjected to such unusual conditions. For example, various parts of missile guidance or propulsion systems must be able to perform reliably at extreme temperatures. Development of these and other technological areas has resulted in recognition that a magnetic material having one easy direction of magnetization would be of value, particularly where this property could be utilized at low temperatures.

A principal object of this invention is to provide magnets having one easy direction of magnetization.

Another object of this invention is to provide a process for producing magnets having one easy direction of magnetization.

Other objects and advantages will be in part obvious and in part explained by reference to the accompanying specification and drawings.

Fig. 1 shows a hysteresis loop illustrating the magnetic characteristic of the usual type of permanent magnet.

Fig. 2 shows a shifted hysteresis loop illustrating the magnetic properties of a magnet made according to the present invention.

Fig. 3 shows a hysteresis loop illustrating the magnetic properties of a magnet made according to the present invention but without a magnetic field being applied.

Generally, this invention concerns permanent magnets and processes for producing permanent magnets having one easy direction of magnetization, which magnets comprise bodies made of (a) alloys consisting of from about 20 to 45 weight percent manganese combined with one or some combination of the metals, iron, nickel and cobalt, other than the iron-manganese binary alloys, and (b) alloys consisting of about 75 to 85 weight percent iron, balance substantially all aluminum.

The process generally comprises preparing a suitable

## 2

alloy body and cooling the quenched alloy in a magnetic field to a temperature sufficiently low to create the one easy direction of magnetization within the alloy body.

It has been mentioned previously that existing alloy magnets have at least two easy directions of magnetization and also have two equivalent stable positions in an applied magnetic field.

A hysteresis loop 10 characteristic of these magnets is shown in Fig. 1, in which the magnetizing field  $H$ , in oersteds, is the axis of the abscissa and the magnetization or  $M$ , in gauss, is the axis of the ordinate. As the field is increased from 0 to higher values of  $H$  in what for convenience may be referred to as the positive direction, the magnetization ( $M$ ) of the material reaches a maximum value  $+M_{max}$  for a given field. If the field  $+H$  is removed, the value of  $+M_{max}$  decreases along the demagnetization curve 11 to  $+M_R$ . If then a field  $-H$  of reverse polarity is applied, the magnetization of the material continues to decrease along curve 11 and crosses the  $H$  axis at the value  $-H_c$ , the magnetization finally reaching  $-H_{max}$  as the field is further increased in the negative direction. If the negative field is removed, the magnetization of the material correspondingly drop to  $-M_R$ , which is numerically equal to  $+M_R$ . Application of the positive field, then causes the magnetization to move along the magnetization curve 12 and cross the  $H$  axis at the value  $+H_c$ , which is numerically equal to  $-H_c$ . As the positive field is increased, the magnetization of the material rises to the value  $+M_{max}$ . The magnetization values  $M$  which were used in the present case in place of the flux density,  $B$ , to plot the hysteresis loops, are equal to the flux density ( $B$ ) minus the magnetizing field ( $H$ ), divided by  $4\pi$ , as indicated by the formula  $M=(B-H)/4\pi$ .

Alloys which can be used, according to the present invention, to produce magnets having one easy direction of magnetization fall generally into two categories. The first category includes alloys containing between 20 and 45 percent manganese and the balance a metal selected from the group consisting of iron, nickel, cobalt and combinations thereof, other than iron-manganese binary alloys. The iron-manganese binary alloys cannot be processed to produce satisfactory results. The second general category of alloys are iron base alloys containing 75 to 85 weight percent of iron and the balance substantially all aluminum.

Fig. 2 shows a hysteresis loop 15 which is characteristic of the magnets of the present invention. Here the loop is shifted toward the negative direction of field, the material thus being more easily magnetized in the positive direction. The maximum fields  $-H_{max}$  and  $+H_{max}$  are quantitatively the same, 8000 oersteds, but the magnetization values  $M_R$  are both positive and the field strengths  $H_c$  are both negative. For purposes of discussion, the magnetization and field values found on the demagnetization curve 16 of the loop are designated  $M_{R1}$  and  $H_{C1}$ , respectively, and the corresponding values on the magnetization curve 17 are designated  $M_{R2}$  and  $H_{C2}$ , respectively.

To illustrate more fully the type of alloys which can be processed to develop the desired properties, several examples follow. First, alloys containing from about 20 to about 35 percent manganese, balance substantially all nickel can be processed to develop the properties resulting in a hysteresis loop. Table I sets forth specific alloy compositions within the previously stated ranges and shows the magnetization and field values obtained at  $4.2^\circ K$ . The table also sets forth the approximate temperature at which the shifted loop effect appears when the various alloys are cooled.

3  
Table I

| Composition, Weight Percent |    | M <sub>R1</sub> (EMU) | M <sub>R2</sub> (EMU) | H <sub>C1</sub> (OE) | H <sub>C2</sub> (OE) | Max. Temp. of Effect, °K. |
|-----------------------------|----|-----------------------|-----------------------|----------------------|----------------------|---------------------------|
| Ni                          | Mn |                       |                       |                      |                      |                           |
| 80                          | 20 | +260                  | +240                  | -200                 | -150                 | 20                        |
| 75                          | 25 | +95                   | +95                   | -500                 | -400                 | 50                        |
| 70                          | 30 | +7                    | +7                    | -6,200               | -5,700               | 80                        |
| 65                          | 35 | +0.5                  | +0.5                  | -2,000               | -2,000               | 90                        |

Additional alloys are those made up of 25 percent manganese, 19 to 37½ percent iron and a balance substantially all nickel. Some specific compositions within these compositional ranges and having desired magnetic properties, are found in the following Table II.

Table II

| Composition, Weight Percent |      |    | M <sub>R1</sub> (EMU) | M <sub>R2</sub> (EMU) | H <sub>C1</sub> (OE) | H <sub>C2</sub> (OE) | Max. Temp. of Effect, °K. |
|-----------------------------|------|----|-----------------------|-----------------------|----------------------|----------------------|---------------------------|
| Ni                          | Fe   | Mn |                       |                       |                      |                      |                           |
| 56                          | 19   | 25 | +235                  | +235                  | -700                 | -600                 | 80                        |
| 50                          | 25   | 25 | +145                  | +145                  | -1,300               | -1,150               | 60                        |
| 37.5                        | 37.5 | 25 | +53                   | +51                   | -4,500               | -3,100               | 45                        |

Cobalt may be totally or partially substituted for nickel and combined with manganese to produce alloys which, when properly processed, have the desired one easy direction of magnetization. The cobalt is added in amounts ranging from 55 to 75 percent in the binary alloys and in amounts up to about 75 percent in the nickel-cobalt-manganese ternary alloys having 25 percent manganese. Table III lists the magnetic characteristics of some of these alloy compositions. It will be noted that in the alloys where cobalt has been substituted for nickel, the field strength (H<sub>C1</sub> and H<sub>C2</sub>) are smaller and also that the temperatures at which the shifted loop characteristic disappears are generally somewhat lower.

Table III

| Composition, Weight Percent |    | M <sub>R1</sub> (EMU) | M <sub>R2</sub> (EMU) | H <sub>C1</sub> (OE) | H <sub>C2</sub> (OE) | Max. Temp. of Effect, °K. |
|-----------------------------|----|-----------------------|-----------------------|----------------------|----------------------|---------------------------|
| Co                          | Mn |                       |                       |                      |                      |                           |
| 70                          | 30 | +28                   | +14                   | -360                 | -130                 | 25                        |
| 65                          | 35 | +4                    | +2                    | -150                 | -50                  | 75                        |
| 60                          | 40 | +2                    | 0                     | -125                 | 0                    | 20                        |
| 55                          | 45 | +2                    | -0.5                  | -125                 | +25                  | 10                        |

As a final compositional illustration, iron and aluminum can be combined in amounts from 75 to 85 weight percent iron and the balance aluminum to obtain an alloy having one easy direction of magnetization. Here, as shown in Table IV, the shift is quite large for some alloy compositions although the temperature at which the effect during cooling appears is generally lower than that for the alloys containing manganese.

Table IV

| Composition, Atomic Percent |    | M <sub>R1</sub> (EMU) | M <sub>R2</sub> (EMU) | H <sub>C1</sub> (OE) | H <sub>C2</sub> (OE) | Max. Temp. of Effect, °K. |
|-----------------------------|----|-----------------------|-----------------------|----------------------|----------------------|---------------------------|
| Fe                          | Al |                       |                       |                      |                      |                           |
| 70                          | 30 | +155                  | -125                  | -700                 | +200                 | 10                        |
| 65                          | 35 | +9                    | +7.5                  | -4,000               | -3,400               | 10                        |
| 60                          | 40 | +2                    | +2                    | -2,700               | -2,400               | 10                        |

As has already been stated, the treatment to which the alloys must be subjected is important in achieving magnets having the magnetic properties evidenced by the

shifted hysteresis loops. In the case of the manganese containing alloys, that is those alloys made up of manganese and one or more of the members iron, nickel, cobalt, and combinations thereof, it is felt that both atomic and magnetic heterogeneity must exist to develop the one easy direction of magnetization. That is, some degree of disorder should exist to bring about the shifted hysteresis loop characteristic, although complete disorder is probably not essential as some ordered regions may exist in almost all systems if only on a statistical basis.

As generally understood, a disordered solid solution alloy is one in which the atoms of the various constituent metals of an alloy are randomly distributed through the alloy lattice. Conversely, an ordered solid solution alloy is one in which the atoms of the different metals repeat in lattice position according to a definite pattern.

The compositions in which ordering must be considered are principally those in which the metals are combined in stoichiometric proportions. For example, ordering would ordinarily occur in the compositions Ni<sub>3</sub>Mn or NiMn. Of course, it is to be understood that the discussion concerning the order or disorder of the various alloys is advanced as a possible explanation of why the effect is seen in these alloys and that other factors may be equally important.

Broadly, the process involves preparing a magnet body of a suitable alloy such as one of those previously disclosed, quenching the body from an elevated temperature to retain some degree of atomic disorder and cooling the body to below about 80° K. in a magnetic field. The temperature to which the body must be cooled in a magnetic field must be equal to or lower than the temperature at which the shifted hysteresis loop effect appears to obtain the one easy direction of magnetization.

In order to obtain optimum properties, the field should be maintained down to the lowest temperature to which the body is cooled. Examples of such temperatures are set forth in Tables I through IV.

In those alloys where ordering is anticipated, the magnet body should be heated to a temperature above 700° C., preferably about 900° C., and held for a sufficient amount of time to insure that disorder is achieved, for example about 12 hours. Once disordered, the metal is quenched rapidly to room temperature to retain disordering as cooling progresses through the lower temperature ranges. The disordered material is then cooled further to some temperature below about 80° K., in a magnetic field, the exact temperature depending upon the particular alloy, as already noted.

Where ordering is not a material consideration, heating of the body to an elevated temperature and subsequent quenching to room temperature need not be effected, although optimum disorder is assured if these steps are included.

It is felt that the present magnets, as processed, acquire their unique behavior by virtue of ferromagnetic and anti-ferromagnetic regions present within the body. The coupling effect between the ferromagnetic and anti-ferromagnetic regions causes the one easy direction of magnetization. Therefore, during cooling of the body from room temperature it is essential that it be subjected to a magnetic field, one on the order of 5000 oersteds normally being sufficient to properly orient the ferromagnetic

moments in any of the alloys. Of course, lesser fields can be used on some of the alloys and still obtain maximum alignment of the magnetic moments within the magnet. Although the magnetic field need only be applied from just above that temperature at which the shifted loop effect begins, as a matter of expedience it is normally easier to apply the field continuously during the entire cooling treatment.

The effect of cooling the body from room temperature to below the critical temperature without using a magnetic field can be shown by referring to loop 20 of Fig. 3 of the drawings. This loop was obtained from the same material used to obtain curve 15, the difference resulting from the absence of an applied magnetic field during cooling.

The processing of the iron-aluminum alloy is generally the same as that of the previously discussed alloys, although the presence of disorder is not felt to be a consideration as the alloys are normally ordered. As an example, an iron-aluminum alloy containing approximately 17 percent aluminum was annealed for 20 hours at 900° C., quenched from 700° C. in water, and then cooled from room temperature to 1.8° K. in a magnetic field of 5000 oersteds. The measurements were made at the point 1.8° K.; the magnetization M was measured in the direction of the field applied during cooling. The hysteresis loop crossed the H axis at plus 200 and minus 700 oersteds, thereby indicating that asymmetry of the hysteresis loop had taken place.

Thus, the present invention has provided a magnet which is totally metallic containing ferromagnetic and anti-ferromagnetic regions which bring about the one easy direction of magnetization.

What we claim as new and desire to secure by Letters Patent of the United States is:

1. In the process of producing a permanent magnet having one easy direction of magnetization at temperatures below about 80° K., the steps comprising preparing a body composed of an alloy selected from the group consisting of (a) alloys containing from about 20 to 45 weight percent manganese, balance a metal from the group consisting of iron, nickel, cobalt, and combinations thereof, other than iron-manganese binary alloys and

(b) alloys containing from about 75 to 85 weight percent iron balance substantially all aluminum, cooling the alloy body to a temperature below about 80° K., and subjecting the body to a magnetic field during cooling to align the magnetic moments of the ferromagnetic regions and develop the one easy direction of magnetization within the body.

- 5 2. In the process of producing a permanent magnet having one easy direction of magnetization at temperatures below about 80° K. with a body composed of an alloy consisting essentially of from about 20 to 45 weight percent manganese, and the balance a metal selected from the group consisting of iron, nickel, cobalt, and combinations thereof, other than iron-manganese binary alloys, the 10 steps comprising cooling the alloy body to a temperature below about 80° K., and subjecting the body to a magnetic field during cooling to align the magnetic moments of the ferromagnetic regions and develop the one easy direction of magnetization within the body.
- 15 3. A process for producing a permanent magnet having one easy direction of magnetization at temperatures below about 80° K., comprising preparing an alloy ingot consisting essentially of from about 20 to 45 weight percent manganese, and the balance a metal selected from 20 the group consisting of iron, nickel, cobalt, and combinations thereof, other than iron-manganese binary alloys, heating the body to above about 700° C., quenching the 25 alloy body, cooling the alloy body to a temperature below about 80° K., and subjecting the body to a magnetic field during cooling to align the magnetic moments of the ferromagnetic regions and develop the one easy direction of magnetization within the body.
- 30 35

#### References Cited in the file of this patent

#### UNITED STATES PATENTS

|           |                |               |
|-----------|----------------|---------------|
| 1,668,115 | Gumlich        | May 1, 1928   |
| 2,133,291 | Gordon         | Oct. 18, 1938 |
| 2,295,082 | Jonas          | Sept. 8, 1942 |
| 2,382,650 | Nesbitt        | Aug. 14, 1945 |
| 2,859,143 | Nachman et al. | Nov. 4, 1958  |

#### FOREIGN PATENTS

|         |             |              |
|---------|-------------|--------------|
| 280,893 | Switzerland | May 16, 1952 |
|---------|-------------|--------------|